

# United States Patent [19]

Ogawa et al.

[11] Patent Number: 4,476,218

[45] Date of Patent: Oct. 9, 1984

[54] SILVER HALIDE PHOTOGRAPHIC  
LIGHT-SENSITIVE MATERIALS

[75] Inventors: Masashi Ogawa; Kunio Ishigaki;  
Taku Nakamura; Nobuyuki Iwasaki,  
all of Kanagawa, Japan

[73] Assignee: Fuji Photo Film Co., Ltd., Kanagawa,  
Japan

[21] Appl. No.: 388,820

[22] Filed: Jun. 16, 1982

[30] Foreign Application Priority Data

Jun. 16, 1981 [JP] Japan ..... 56-92559

[51] Int. Cl.<sup>3</sup> ..... G03C 1/76; G03C 1/30

[52] U.S. Cl. ..... 430/539; 430/621;  
430/622; 430/961

[58] Field of Search ..... 430/351, 355, 961, 621-626,  
430/539

[56] References Cited

U.S. PATENT DOCUMENTS

3,782,955 1/1974 Mucke et al. ..... 430/351  
3,923,517 12/1975 Yamamoto et al. ..... 430/621  
4,021,248 5/1977 Shiba et al. ..... 430/351

4,161,407 7/1979 Campbell ..... 430/621  
4,264,721 4/1981 Shimano et al. ..... 430/351  
4,267,265 5/1981 Sugimoto et al. ..... 430/961  
4,304,852 12/1981 Sugimoto et al. ..... 430/961  
4,366,238 12/1982 Yokoyama et al. ..... 430/961

FOREIGN PATENT DOCUMENTS

1534455 11/1978 United Kingdom .

Primary Examiner—Mary F. Downey  
Attorney, Agent, or Firm—Sughrue, Mion, Zinn,  
Macpeak and Seas

[57]

ABSTRACT

A silver halide photographic light-sensitive material is described, which comprises a support, and at least one light-sensitive silver halide emulsion layer and an uppermost layer provided on at least one surface of the support, wherein the melting time of the uppermost layer is made greater than that of the light-sensitive silver halide emulsion layer. The material has good strength and produces a reduced amount of scum which normally occurs in the processing liquid during development processing.

12 Claims, No Drawings

SILVER HALIDE PHOTOGRAPHIC  
LIGHT-SENSITIVE MATERIALS

## FIELD OF THE INVENTION

The present invention relates to silver halide photographic light-sensitive materials. More particularly, it is concerned with silver halide photographic light-sensitive materials which form less scum in processing liquids and can be rapidly processed at high temperatures.

## BACKGROUND OF THE INVENTION

It has been greatly desired to shorten the time required for development of light-sensitive materials. In order to meet these requirements, the development time has been reduced by raising the development temperature to about 27° C. or higher. This is realized by the use of an automatic developing machine as described in, e.g., *Rodal Technol.*, Vol. 44, No. 4, pp. 257-261 (1973), U.S. Pat. Nos. 3,025,779 and 3,672,288 which permits rapid and highly reproducible development. Such automatic developing machines usually contain a developing tank, a stopping tank, a fixing tank, a water-washing tank, a drying zone, and so forth, and the speed of conveyance of films and the processing temperature can be controlled.

It is known, as described in Furnell et al., *J. Photo. Sci.*, Vol. 18, p. 94 (1970), that with photographic light-sensitive materials using a silver halide emulsion, when the degree of swelling of the material in a developer is changed by changing the degree of hardening of a binder, e.g., gelatin, the covering power based on developed silver can be increased. It has been observed that as the degree of hardening of a silver halide emulsion layer is decreased by reducing the amount of a hardener used, the covering power is further increased.

However, when the degree of hardening is lowered to great extent, the strength of the emulsion layer is seriously reduced, presenting various problems. For example, when processed in an automatic developing machine as described hereinbefore, the emulsion layer is liable to peel apart from the support, or it may be readily scratched during the handling. Furthermore, binders may come out of the light-sensitive materials into the processing liquids in the automatic developing machine. These binders may combine together with each other, or with different compounds from the light-sensitive material in the processing liquid, and form precipitates insoluble in the processing liquid. These insoluble precipitates in the processing liquids are generally called "scum" in the art.

When scum is formed in a processing liquid, it sticks to a light-sensitive material which later passes through the automatic developing machine, causing contamination of the light-sensitive material. The scum sticking to the light-sensitive material seriously deteriorates the image quality of the light-sensitive material, as a result of which the product value is completely lost.

In order to overcome such problems, it is necessary to increase the degree of hardening of a silver halide emulsion layer to some extent. However, this inevitably leads to a reduction in the covering power. Although a number of methods for hardening silver halide emulsion layers are known, none of these methods make it possible to increase covering power without causing the formation of scum in processing liquids.

As a result of extensive studies to solve the above-described problems, it has been found that by control-

ling the degree of hardening of the uppermost layer independently from those of other underlying layers, i.e., by making the former greater than the latter, the elution of gelatin can be prevented. Accordingly, the formation of scum can be greatly reduced. Although it is well known that unreacted gelatin which has not been cross-linked by a hardener comes out from a light-sensitive material, and that the amount of the unreacted gelatin depends on the degree of hardening, it has been found for the first time according to the present invention that when the degree of hardening of the uppermost layer is increased, even if the degrees of hardening of underlying layers are small, i.e., the proportion of cross-linked gelatin in each of the underlying layers is small, the amount of gelatin eluted can be greatly reduced compared with conventional light-sensitive materials in which the degree of hardening of gelatin is the same in all coating layers. Furthermore, astonishingly, it has been found that the amount of gelatin eluted is based almost totally on the degree of hardening of the uppermost layer and is less affected by the degrees of hardening of the other underlying layers. This indicates that the cross-linking of the uppermost layer produces synergistic effects in the prevention of elution of gelatin. These synergistic effects could not have been anticipated by prior art teachings.

## SUMMARY OF THE INVENTION

The object of the invention is to provide silver halide photographic light-sensitive materials which have a high covering power and when processed in an automatic developing machine, do not produce any scum in processing liquids in the automatic developing machine.

The present invention, therefore, relates to a silver halide photographic light-sensitive material comprising a support with at least one light-sensitive silver halide emulsion layer and the uppermost layer on at least one side thereof wherein the "melting time" of the uppermost layer is greater than that of the light-sensitive silver halide emulsion layer. The melting time (MT) is discussed further below and relates to the time required for a hardened layer to melt when it is soaked in a solution maintained at a certain temperature.

DETAILED DESCRIPTION OF THE  
INVENTION

As is known in the art, the degree of hardening can be controlled from layer to layer by the use of non-diffusible hardeners. As such non-diffusible hardeners, various polymeric hardeners which have molecular weight of more than about 10,000 and at least one functional group reactive to gelatin to form cross-linking can be used in the silver halide photographic light-sensitive materials of the present invention. These hardeners include those as described in, for example, U.S. Pat. Nos. 3,057,723, 3,396,029, 4,161,407, British Pat. No. 2,064,800 and U.S. application Ser. No. 251,827. One preferred example of the polymeric hardener is that described in U.S. application Ser. No. 251,827, which has a repeating unit represented by the following formula (I):



wherein A is a monomer unit prepared by copolymerizing copolymerizable ethylenically unsaturated monomers; R<sub>1</sub> is hydrogen or a lower alkyl group having 1 to 6 carbon atoms; Q is —CO<sub>2</sub>—,



(wherein R<sub>1</sub> is the same as defined above) or an arylene group having 6 to 10 carbon atoms; L is a divalent group having 3 to 15 carbon atoms and containing at least one linking group selected from the members consisting of —CO<sub>2</sub>— and



(wherein R<sub>1</sub> is the same as defined above) or a divalent group having 1 to 12 carbon atoms and containing at least one linking group selected from the members consisting of —O—,



—CO—, —SO—, —SO<sub>2</sub>—, —SO<sub>3</sub>—,



(wherein R<sub>1</sub> is the same as defined above); R<sub>2</sub> is —CH=CH<sub>2</sub> or —CH<sub>2</sub>CH<sub>2</sub>X (wherein X is a group capable of being substituted with a nucleophilic group or a group capable of being released in the form of HX upon a base; and x and y each represents molar percent, x being between 0 and 99 and y being between 1 and 100.

Examples of ethylenically unsaturated monomers represented by "A" of formula (I) include ethylene, propylene, 1-butene, isobutene, styrene, chloromethylstyrene, hydroxymethylstyrene, sodium vinylbenzenesulfonate, sodium vinylbenzylsulfonate, N,N,N-trimethyl-N-vinylbenzylammonium chloride, N,N-dimethyl-N-benzyl-N-vinylbenzylammonium chloride,  $\alpha$ -methylstyrene, vinyltoluene, 4-vinylpyridine, 2-vinylpyridine, benzyl vinylpyridinium chloride, N-vinylacetamide, N-vinylpyrrolidone, 1-vinyl-2-methylimidazole, monoethylenically unsaturated esters of aliphatic acids (e.g., vinyl acetate and allyl acetate), ethylenically unsaturated mono- or dicarboxylic acids and salts thereof (e.g., acrylic acid, methacrylic acid, itaconic acid, maleic acid, sodium acrylate, potassium acrylate and sodium methacrylate), maleic anhydride, esters of ethylenically unsaturated monocarboxylic or dicarboxylic acids (e.g., n-butyl acrylate, n-hexyl acrylate, hydroxyethyl acrylate, cyanoethyl acrylate, N,N-diethylaminethyl acrylate, methyl methacrylate, n-butyl methacry-

late, benzyl methacrylate, hydroxyethyl methacrylate, chloroethyl methacrylate, methoxyethyl methacrylate, N,N-diethylaminoethyl methacrylate, N,N,N-triethyl-N-methacryloyloxyethylammonium-p-toluene sulfonate, N,N-diethyl-N-methyl-N-methacryloyloxyethylammonium-p-toluene sulfonate, dimethyl itaconate and monobenzyl maleate), and amides of ethylenically unsaturated monocarboxylic or dicarboxylic acids (e.g., acrylamide, N,N-dimethylacrylamide, N-methylolacrylamide, N-(N,N-dimethylaminopropyl)acrylamide, N,N,N-trimethyl-N-(N-acryloylpropyl)ammonium-p-toluene sulfonate, sodium 2-acrylamide-2-methylpropane sulfonate, acryloyl morpholine, methacrylamide, N,N-dimethyl-N'-acryloyl propane diamine propionate betaine, and N,N-dimethyl-N'-methacryloyl propane diamine acetate betaine). "A" further includes monomers having at least two copolymerizable ethylenically unsaturated groups (e.g., divinylbenzene, methylenesacrylamide, ethylene glycol diacrylate, trimethylene glycol diacrylate, ethylene glycol dimethacrylate, trimethylene glycol dimethacrylate and neopentyl glycol dimethacrylate).

Examples of R<sub>1</sub> of formula (I) include a methyl group, an ethyl group, a butyl group and an n-hexyl group.

Examples of Q of formula (I) include the following groups: —CO<sub>2</sub>—, —CONH—,



35



Examples of L of formula (I) include the following groups: —CH<sub>2</sub>CO<sub>2</sub>CH<sub>2</sub>—, —CH<sub>2</sub>CO<sub>2</sub>CH<sub>2</sub>CH<sub>2</sub>—, —CH<sub>2</sub>CH<sub>2</sub>CO<sub>2</sub>CH<sub>2</sub>CH<sub>2</sub>—, —(CH<sub>2</sub>)<sub>5</sub>CO<sub>2</sub>CH<sub>2</sub>CH<sub>2</sub>—, —(CH<sub>2</sub>)<sub>10</sub>CO<sub>2</sub>CH<sub>2</sub>CH<sub>2</sub>—, —CH<sub>2</sub>NHCOCH<sub>2</sub>—, —CH<sub>2</sub>NHCOCH<sub>2</sub>CH<sub>2</sub>—, —(CH<sub>2</sub>)<sub>3</sub>NHCOCH<sub>2</sub>C<sub>6</sub>H<sub>5</sub>—, —(CH<sub>2</sub>)<sub>5</sub>NHCOCH<sub>2</sub>CH<sub>2</sub>—, —(CH<sub>2</sub>)<sub>10</sub>NHCOCH<sub>2</sub>CH<sub>2</sub>—, —CH<sub>2</sub>OCH<sub>2</sub>—, —CH<sub>2</sub>C<sub>6</sub>H<sub>5</sub>OCH<sub>2</sub>CH<sub>2</sub>CH<sub>2</sub>—,

55



—COCH<sub>2</sub>CH<sub>2</sub>—, —CH<sub>2</sub>COCH<sub>2</sub>CH<sub>2</sub>—,

60



—SOCH<sub>2</sub>CH<sub>2</sub>—, —CH<sub>2</sub>SOCH<sub>2</sub>CH<sub>2</sub>—, —SO<sub>2</sub>CH<sub>2</sub>C<sub>6</sub>H<sub>5</sub>—, —SO<sub>2</sub>CH<sub>2</sub>CH<sub>2</sub>SO<sub>2</sub>CH<sub>2</sub>CH<sub>2</sub>—,

65



5



Examples of  $\text{R}_2$  of formula (I) include the following groups:  $-\text{CH}=\text{CH}_2$ ,  $-\text{CH}_2\text{CH}_2\text{Cl}$ ,  $-\text{CH}_2\text{CH}_2\text{Br}$ ,  $-\text{CH}_2\text{CH}_2\text{O}_3\text{SCH}_3$ ,



Another preferred example of the polymeric hardener is that described in U.S. Pat. No. 4,161,407, which has a repeating unit represented by the following formula (II):



(II)

wherein A is a polymerized  $\alpha,\beta$ -ethylenically unsaturated addition polymerizable monomer or a mixture of such polymerizable monomers; x and y are the molar percentages of the resulting units in the polymer and are whole integers, x being from 10 to about 95 percent and y being 5 to 90 percent; R is hydrogen or an alkyl group having 1 to 6 carbon atoms; R' is  $-\text{CH}=\text{CHR}_2$  or  $-\text{CH}_2\text{CH}_2\text{X}$  where X is a leaving group which is displaced by a nucleophile or eliminated in the form of HX by treatment with base; R<sub>2</sub> is alkyl, aryl or hydrogen; L is a linking group selected from the group consisting of alkylene, preferably containing about 1 to 6 carbon atoms, such as methylene, ethylene, isobutylene and the like; arylene of about 6 to 12 nuclear carbon atoms, such as phenylene, tolylene, naphthalene and the like;  $-\text{COZ}$  or  $-\text{COZR}_3$ ; R<sub>3</sub> is alkylene, preferably of 1 to 6 carbon atoms, or arylene, preferably of 6 to 12 carbon atoms; and Z is O or NH.

Examples of A of formula (II) include the same examples of A of formula (I), examples of R of formula (II) include the same examples of R<sub>1</sub> of formula (I) and examples of R' of formula (II) include the same examples of R<sub>2</sub> of formula (I), all of which are described above.

Still another preferred example of the polymeric hardener is that described in British Pat. No. 1,534,455, which has a repeating unit represented by the following formula (III):



(III)

wherein A is a monomer unit copolymerized with a copolymerizable ethylenically unsaturated monomer; R is a hydrogen atom or an alkyl group having 1 to 6 carbon atoms; L is a divalent linking group having 1 to 20 carbon atoms; X is an active ester group; x and y each represents molar percent, with x being between 0 and 95 and y being between 5 and 100 and m is 0 or 1.

Examples of A of formula (III) include the same examples of A of formula (I) and examples of R of formula (III) include the same examples of R<sub>1</sub> of formula (I), both of which are described above.

Examples of L of formula (III) include the following:



Examples of X of formula (III) include the following:

30





15 Among the above preferred examples of the polymeric hardeners, the polymeric hardener having repeating unit of formula (I) is particularly preferred.

Typical examples of the polymeric hardener are shown below as P-1 to P-22. Among them, P-1, 2, 6 and 19 are particularly preferred.



$x/y = 3/1$



$x/y = 3/1$



$x/y = 3/1$



$x/y = 3/1$



$x/y = 3/1$



$x/y = 3/1$



$x/y = 3/1$

-continued



x/y = 3/1



x/y = 3/1



x/y = 3/1



x/y = 3/1



-continued



x/y = 3/1



x/y = 3/1



x/y = 3/1



x/y = 3/1



x/y = 3/1

In the above formulae, M is a hydrogen atom, a sodium atom or a potassium atom, and x and y represent the molar percent of the corresponding units charged. The molar percent is not limited to those specified in the above formulae, x may be from 0 to 99, and y, from 1 to 100.

Usually, the polymeric hardener of the present invention is used in an amount such that it contains from  $0.1 \times 10^{-3}$  to  $30 \times 10^{-3}$  equivalent of functional group reactive to gelatin per 100 g of gelatin. A particularly preferable range is from  $0.5 \times 10^{-3}$  to  $10 \times 10^{-3}$  equivalent per 100 g of gelatin.

Methods of synthesizing typical ethylenically unsaturated monomers containing a vinyl sulfone group or its precursor which are used in the preparation of polymeric hardeners for use in the invention will hereinafter be described.

#### PREPARATION EXAMPLE 1

##### Synthesis of 2-[3-(Chloroethylsulfonyl)propionyloxy]ethyl Acrylate

A mixture of 600 ml of tetrahydrofuran, 45.8 g of hydroxyethyl acrylate, and 72 g of 3-(2-chloroethylsulfonyl)propionic acid chloride was placed in a reactor, and while maintaining the temperature at 5°C. or lower by cooling by ice water, a solution of 31.2 g of pyridine in 100 ml of tetrahydrofuran was added dropwise thereto over a period of 1.75 hours. The resulting mixture was further stirred for 2 hours at room tempera-

40

ture. At the end of the time, the reaction mixture was poured into 2,500 ml of ice water, and extraction was performed four times with 300 ml of chloroform. The organic layer thus extracted was dried over sodium sulfate and concentrated to provide 87 g of 2-[3-(chloroethylsulfonyl)propionyloxy]ethyl acrylate. Yield was 88%.

#### PREPARATION EXAMPLE 2

##### Synthesis of [3-(Chloroethylsulfonyl)propionyl]aminomethylstyrene

A mixture of 100 ml of tetrahydrofuran, 20.1 g of vinylbenzylamine, 16.7 g of triethylamine, and 0.1 g of hydroquinone was placed in a reactor, and while cooling with ice water, a solution of 36.1 g of  $\beta$ -chloroethylsulfonylpropionic acid chloride in 200 ml of tetrahydrofuran was added dropwise thereto over a period of 30 minutes. The resulting mixture was allowed to stand overnight at room temperature. The reaction mixture was then poured into a solution prepared by diluting 16.5 g of concentrated hydrochloric acid with 1,500 ml of ice water, and a precipitate was filtered off. The precipitate was recrystallized from a mixed solvent of 200 ml of ethanol and 200 ml of water to provide 26.8 g of N-vinylbenzyl- $\beta$ -chloroethylsulfonyl propionic acid amide. Yield was 57%. Elemental analysis (found): H, 5.74; C, 53.47; N, 4.83; Cl, 10.99; S, 10.49.

50

45

50

55

60

65

## PREPARATION EXAMPLE 3

## Synthesis of

1-[2-(4-Vinylbenzenesulfonyl)ethyl]sulfonyl]-3-chloroethylsulfonyl-2-propanol

A mixture of 157 g of 1,3-bischloroethylsulfonyl-2-propanol (prepared by the method disclosed in British Pat. No. 1,534,455), 1,000 ml of methanol, and 1,000 ml of distilled water was placed in a reactor, and while maintaining the temperature at 46° C., a solution prepared by dissolving 52 g of potassium vinylbenzenesulfonate in 100 ml of methanol and 100 ml of distilled water was added dropwise thereto over a period of 1 hour. The resulting mixture was further stirred for 5.5 hours while maintaining at 46° C. The precipitate thus formed was filtered off to obtain 55 g of 2-(1-vinylbenzenesulfonyl)ethylsulfonyl-3-chloroethylsulfonyl-2-propanol. Yield was 49%. Elemental analysis (found): H, 4.67; C, 39.89; S, 21.43.

## PREPARATION EXAMPLE 4

## Synthesis of

N-[3-(Vinylsulfonyl)propionyl]aminomethyl-acrylamide

In a 2,000 ml reactor were introduced 1,400 ml of distilled water, 224 g of sodium sulfite, and 220 g of sodium hydrogencarbonate, which were then stirred to form a uniform solution. Then, while maintaining the temperature of about 5° C. by cooling with ice water, 260 g of chloroethanesulfonyl chloride was added dropwise thereto over a period of 1.5 hours. After the dropwise addition was completed, 160 g of 49% sulfuric acid was added dropwise thereto over a period of about 15 minutes, and the resulting mixture was stirred for 1 hour at 5° C. Crystals precipitated were collected by filtration and washed with 400 ml of distilled water. The filtrate and the washing liquid were combined together and placed in a 3,000 ml reactor. Into the reactor was introduced dropwise a solution of 246 g of methylenebisacrylamide in 480 ml of distilled water and 1,480 ml of ethanol while maintaining the temperature at about 5° C. over a period of 30 minutes. The reactor was then placed in a refrigerator and was allowed to stand for 5 days to complete the reaction. Crystals precipitated were collected by filtration and, thereafter, they were washed with 800 ml of distilled water and recrystallized from 2,000 ml of a 50% aqueous solution of ethanol to obtain 219 g of the desired monomer. Yield was 49%.

In addition, methods of synthesizing polymeric hardeners which are preferably used in the present invention will hereinafter be described.

## PREPARATION EXAMPLE 5

Synthesis of 2-[3-(Vinylsulfonyl)propionyloxy]ethyl Acrylate/Sodium Acrylamido-2-methylpropanesulfonate Copolymer (P-1)

A mixture of 60 ml of N,N-dimethylformamide, 14.5 g of 2-[3-(chloroethylsulfonyl)propioyloxy]ethyl acrylate, and 23.5 g of acrylamido-2-methylpropanesulfonic acid was placed in a reactor. After purging with nitrogen gas, the mixture was heated to 60° C., and 0.40 g of 2,2'-azobis(2,4-dimethylvaleronitrile) was added thereto. The resulting mixture was stirred for 2 hours while heating at that temperature. Subsequently, 0.2 g of 2,2'-azobis(2,4-dimethylvaleronitrile) was added, and the mixture was stirred for 2 hours while heating. At the

end of the time, the mixture was cooled down to 5° C., and 12 g of sodium carbonate and 4.9 g of triethylamine were added. The resulting mixture was stirred for 1 hour and additionally for 1 hour at room temperature. The reaction mixture was placed in a tube of cellulose and was subjected to dialysis for 2 days. The product was freeze-dried to obtain 35 g of a white polymer. Yield was 95%. The vinylsulfone content of the polymer thus formed was  $0.51 \times 10^{-3}$  equivalent/g.

## PREPARATION EXAMPLE 6

## Synthesis of

[3-(Chloroethylsulfonyl)propionyl]aminomethyl-styrene/Sodium Acrylamido-2-methylpropanesulfonate Copolymer (P-6)

A mixture of 15.8 g of [3-(Vinylsulfonyl)propionyl]aminomethylstyrene, 23.6 g of sodium acrylamido-2-methylpropanesulfonate, and 75 ml of N,N-dimethylformamide was placed in a reactor. After purging with nitrogen gas, the mixture was heated to 80° C., and 0.75 g of 2,2'-azobis(2,4-dimethylvaleronitrile) was added thereto. The resulting mixture was stirred for 3 hours while heating. Then, 25 ml of N,N-dimethylformamide was added, and subsequently 6.1 g of triethylamine was added dropwise at room temperature. The resulting mixture was stirred for 1 hour at room temperature. At the end of the time, the reaction mixture was filtered. The filtrate thus obtained was poured into 800 ml of acetone, and the thus-formed precipitate was filtered off and dried to obtain 36.2 g of pale yellow polymer. Yield was 94%. The vinylsulfone content of the polymer was  $0.80 \times 10^{-3}$  equivalent/g.

## PREPARATION EXAMPLE 7

## Synthesis of

1-[2-(4-Vinylbenzenesulfonyl)ethyl]sulfonyl]-3-chloroethylsulfonyl-2-propanol/Sodium Acrylate Copolymer (P-19)

A mixture of 300 ml of N,N-dimethylformamide, 40.1 g of 2-(1-vinylbenzenesulfonyl)ethylsulfonyl-3-chloroethylsulfonyl-2-propanol, and 13.0 g of acrylic acid was placed in a reactor. After purging with nitrogen gas, the mixture was heated to 70° C., and 0.53 g of 2,2'-azobis(2,4-dimethylvaleronitrile) was added thereto. The resulting mixture was heated for 1.5 hours while stirring. Subsequently, 0.53 g of 2,2'-azobis(2,4-dimethylvaleronitrile) was added thereto, and the mixture was further heated for 1 hour while stirring. The reaction mixture was allowed to cool down to room temperature, and 54.8 g of a 28% methanol solution of sodium methylate was added dropwise thereto. Stirring was further continued for 1 hour. The reaction mixture was placed in a tube of cellulose and was subjected to dialysis for 2 days. The product was freeze-dried to obtain 30 g of pale yellow polymer. Yield was 56%. The vinylsulfone content of the polymer was  $1.4 \times 10^{-3}$  equivalent/g.

## PREPARATION EXAMPLE 8

## Synthesis of Polymer (P-2)

A mixture of 5.65 g of the monomer prepared in Preparation Example 1, 9.16 g of sodium acrylamido-2-methylpropanesulfonate, and 80 ml of a 50% aqueous solution of ethanol was placed in a 200 ml reactor, and was heated to 80° C. while stirring. At this temperature,

0.1 g of 2,2'-azobis(2,4-dimethylvaleronitrile) (sold by Wako Pure Chemical Industries Ltd. under the trade name of V-65) was added and additionally, after 30 minutes, 0.1 g of the same compound as above was added. The mixture was heated for 1 hour while stirring. Thereafter, the reaction mixture was cooled down to about 10° C. with ice water, and a solution of 2.5 g of triethylamine in 80 ml of ethanol was added thereto. Stirring was further continued for 1 hour. At the end of the time, the reaction mixture was poured into 1,000 ml of acetone while stirring, and the thus-formed precipitate was filtered off to obtain 12.4 g of Polymer (P-2). Yield was 85%. The intrinsic viscosity,  $[\eta]$ , was 0.227, and the vinylsulfone content was  $0.95 \times 10^{-3}$  equivalent/g.

In hardening emulsion layers, polymeric hardeners as described hereinbefore may be used either singly or in combination with diffusible low-molecular hardeners. Diffusible hardeners which can be used include various organic and inorganic hardeners which are used either singly or in combination with each other. Typical examples of such hardeners include aldehyde compounds, e.g., mucochloric acid, formaldehyde, trimethylolmelamine, glyoxal, 2,3-dihydroxy-1,4-dioxane, 2,3-dihydroxy-5-methyl-1,4-dioxane, succinaldehyde, and glutaraldehyde; active vinyl compounds, e.g., divinyl sulfone, methylenebismaleimide, 1,3,5-triacryloyl-hexahydro-s-triazine, 1,3,5-trivinylsulfonyl-hexahydro-s-triazine, bis(vinylsulfonylmethyl) ether, 1,3-bis(vinylsulfonyl)propanol-2, bis( $\alpha$ -vinylsulfonylacetamido)-ethane, 1,2-bis(vinylsulfonyl)ethane, and 1,1'-bis(vinylsulfonyl)methane; active halogeno compounds, e.g., 2,4-dichloro-6-hydroxy-6-methoxy-s-triazine; and ethyleneimine compounds, e.g., 2,4,6-triethyleneimino-s-triazine. These compounds are well known in the art as hardeners for gelatin.

These polymeric hardeners are dissolved in water or organic solvents and, thereafter, are added directly to a layer in order to control the degree of hardening of that particular layer. In the case of diffusible hardeners, they may be added directly to the layer which is to be controlled in the degree of hardening, or alternatively they may be added to another layer and then diffused in the whole layer. The amount of the non-diffusible hardener added is determined by the amount of the reactive group in the polymeric hardener.

Non-diffusible hardeners may be used either singly or in combination with diffusible hardeners.

In accordance with another technique to control the degrees of hardening of coating layers, low molecular hardeners are employed. By controlling the method of addition and drying conditions, diffusion properties are controlled. For example, a low molecular weight hardener containing a vinylsulfone group is incorporated into only a coating solution for a surface protective layer and, after a plurality of layers are coated at the same time, the layers are rapidly dried whereby the degree of hardening can be changed from layer to layer.

Measures well known in the art for evaluation of the degree of hardening of a hardened layer include the degree of swelling as determined by swelling the hardened layer in a certain solution, and the scratching strength which is indicated by determining the load at which the hardened layer is scratched by a needle-like stylus under the load. However, in order to evaluate the prevention of scum (which is the primary purpose of the present invention), it is most effective to employ a melting time (MT). The melting time is the time required for

a hardened layer to melt when it is soaked in a solution maintained at a certain temperature. It is most preferred to measure the melting time in a 0.2N NaOH solution maintained at 60° C. although the present invention is not limited thereto.

Silver halide emulsions as used herein are ordinarily prepared by mixing water-soluble silver salt (e.g., silver nitrate) solutions and water-soluble halogenide (e.g., potassium bromide) solutions in the presence of water-soluble polymer (e.g., gelatin) solutions.

Silver halides which can be used include mixed silver halides, e.g., silver chlorobromide, silver iodobromide, and silver chloroiodobromide, as well as silver chloride, silver bromide, and silver iodide.

These silver halide grains can be prepared by the usual techniques. It is also useful to prepare them by the so-called single or double jet method, and control double jet method, and so forth.

Photographic emulsions are well known as described in, for example, Mees, *The Theory of Photographic Process*, Macmillan Corp., and P. Glafkides, *Chimie Photographique*, Paul Montel (1957), and can be prepared by various known techniques such as an ammonia method, a neutral method, and an acidic method.

Silver halide emulsions are usually subjected to chemical sensitization although so-called primitive emulsions not subjected to chemical sensitization may be used. Chemical sensitization can be achieved by the methods as described in the above-described reference by P. Glafkides, the book by Zelikman, and H. Frieser Ed., *Die Grundlagen der Photographischen Prozesse mit Silberhalogeniden*, Akademische Verlagsgesellschaft (1968).

A sulfur sensitization method in which compounds containing sulfur capable of reacting with a silver ion, and active gelatin are used, a reduction sensitization method in which reducing compounds are used, a noble metal sensitization method in which gold and other noble metal compounds are used, and so forth can be used either singly or in combination with each other.

Sulfur sensitizers which can be used include thiosulfates, thioureas, thiazoles, and rhodanines. These compounds are described in U.S. Pat. Nos. 1,574,944, 2,410,689, 2,278,947, 2,728,668, 3,656,955, 4,030,928 and 4,067,740. Reduction sensitizers which can be used include stannous salts, amines, hydrazine derivatives, formamidinesulfonic acid, and silane compounds. These compounds are described in U.S. Pat. Nos. 2,487,850, 2,419,974, 2,518,698, 2,983,609, 2,983,610, 2,694,637, 3,930,867 and 4,054,458. For noble metal sensitization, in addition to gold complex salts, complex salts of Group VIII metals, e.g., platinum, iridium, and palladium, of the Periodic Table can be used. These compounds are described in U.S. Pat. Nos. 2,399,083 and 2,448,060, and British Pat. No. 618,061.

Hydrophilic colloids which can be used in the present invention as binders for silver halide include high molecular weight gelatin, colloidal albumin, casein, cellulose derivatives, e.g., carboxymethyl cellulose, and hydroxyethyl cellulose, sugar derivatives, e.g., agar, sodium alginate, and starch derivatives, and synthetic hydrophilic colloids, e.g., polyvinyl alcohol, poly-N-vinylpyrrolidone, polyacrylic acid copolymers, and polyacrylamide, or their derivatives or partially hydrolyzed products. If necessary, mixtures comprising two or more mutually soluble colloids of the above-described compounds may be used. Of the above-described compounds, gelatin is most commonly used.

Part or the whole of gelatin may be displaced by a synthetic polymeric substance. In addition, it may be displaced by a graft polymer prepared by bonding molecular chains of other polymeric substances. Furthermore, gelatin derivatives prepared by treating the usual high molecular weight gelatin with reagents containing a group capable of reacting with an amino group, an imino group, a hydroxy group, or a carboxy group contained in the gelatin may be used partially.

Various compounds may be incorporated into the photographic emulsions used herein for the purpose of preventing the formation of fog during the production of light-sensitive materials or the storage thereof, or of stabilizing photographic performance. Compounds which can be used for that purpose include azoles, e.g., benzothiazolium salts, nitroindazoles, nitrobenzimidazoles, chlorobenzimidazoles, bromobenzimidazoles, mercaptothiazoles, mercaptobenzothiazoles, mercaptobenzimidazoles, mercaptothiadiazoles, aminotriazoles, benzotriazoles, nitrobenzotriazoles, and mercaptotetrazoles (especially, 1-phenyl-5-mercaptop-tetrazole); mercaptopyrimidines; mercaptotriazines; thioketo compounds. e.g., oxazolinethion; azaindenes, e.g., triazaindenes, tetraazaindenes (especially, 4-hydroxy-substituted (1,3,3a,7)tetraazaindenes), and pentaazaindenes; and benzenethiosulfonic acid, benzenesulfonic acid, and benzenesulfonic acid amide, which are known as anti-foggants or stabilizers.

Photographic emulsion layers and other hydrophilic colloid layers in the light-sensitive materials of the present invention may contain various known surfactants as coating aids or for various purposes of prevention of charging, improvement of sliding properties, emulsification and dispersion, prevention of adhesion, and improvement of photographic characteristics (e.g., acceleration of development, high contrast, and sensitization).

Photographic emulsions as used herein may be subjected to spectral sensitization using methine dyes, etc. Dyes which can be used include cyanine dyes, merocyanine dyes, composite cyanine dyes, composite merocyanine dyes, holopolar cyanine dyes, hemicyanine dyes, styryl dyes, and hemioxonol dyes.

Photographic emulsion layers or their adjacent layers in the photographic light-sensitive materials of the present invention may contain, for the purpose of increasing sensitivity, increasing contrast, or for accelerating development, polyalkyleneoxide or its ether, ester, amine or like derivatives, thioether compounds, thiomorpholines, quaternary ammonium chloride compounds, urethane derivatives, urea derivatives, imidazole derivatives, 3-pyrazolidones, and the like.

There are no limitations on surfactants, chemical sensitizers, silver halide, stabilizers, anti-foggants, anti-static agents, matting agents, spectral sensitizing dyes, dyes, color couplers, supports, and so forth, which are used in the silver halide emulsion layers and other hydrophilic colloid layers of the present invention. These additives are described in, for example, *Research Disclosure*, Vol. 176, pp. 22-31 (Dec. 1978) and Japanese Patent Application (OPI) No. 99928/78 (the term "OPI" as used herein refers to a "published unexamined Japanese patent application").

The light-sensitive material of the present invention is characterized in that the uppermost layer lying on a silver halide emulsion layer has a melting time longer than that of the silver halide emulsion layer.

The relation between the melting time of the uppermost layer (MTu) and that of the light-sensitive silver halide emulsion layer (MTs) employed in the present invention can be represented by MTu/MTs ratio. The ratio is usually in a range of more than 1 and less than 20, preferably more than 1 and less than 10, and most preferably more than 3 and less than 6.

The silver halide light-sensitive photographic materials of the present invention may include those having at least one of the light-sensitive silver halide emulsion layer on both sides of the support and the uppermost layer on the outside of the outermost silver halide emulsion layer existed on both sides of the support.

The uppermost layer existed in the silver halide light-sensitive photographic material of the present invention has a thickness of from about 0.5 to about 2.0 microns.

If necessary, a gelatin overcoat layer may be provided on the uppermost layer. It is preferred for such overcoat layers to have melting times shorter than that of the emulsion layer and to be as thin as possible. The gelatin overcoat layer described above should have a thickness of less than 0.5 microns.

A method of exposure of the light-sensitive material of the invention is not critical, and the exposure time may be either as long as from 1 second to several minutes or as short as from  $10^{-6}$  to  $10^{-3}$  second.

Preferred examples of automatic developing machines which can be used in the development of the light-sensitive material of the present invention include a roller conveyor type automatic developing machine, a belt conveyor type automatic developing machine, and a hanger type automatic developing machine. The development process temperature is preferably from 20° to 60° C. and more preferably from 27° to 45° C., and the development time is preferably from 10 seconds to 10 minutes and more preferably from 20 seconds to 5 minutes. Development processing steps, the composition of processing liquids, and so forth may be chosen referring to the above-described references and also to C. E. K. Mees & T. H. James, *The Theory of Photographic Processes*, 3rd Ed., Chapter 13, Macmillan Co. (1966) and L. F. A. Mason, *Photographic Processing Chemistry*, pp. 16-30, Oxford Press (1966).

The following examples are given to illustrate the invention in greater detail.

#### EXAMPLE 1

On both surfaces of an about  $175\mu$  thick polyethylene terephthalate film support which had been coated with a subbing layer on both surfaces were coated an emulsion layer and a protective layer having the formulations as shown below in that sequence to prepare Samples 1 to 8.

In Samples 1 to 8, a hardener as shown in Table 1 was added to each layer.

##### Emulsion Layer

Binder: 2.0 g/m<sup>2</sup> Gelatin  
Amount of Silver Halide: 3.91 g/m<sup>2</sup>  
Composition of Silver Halide: 2.0 mol% AgI + 98.0 mol% AgBr

Anti-Foggant: 0.5 g/Ag 100 g 1-Phenyl-5-mercaptotetrazole and 0.8 g/Ag 100 g 4-hydroxy(1,3,3a,7)tetraazaindene

##### Protective Layer

Binder: 1.3 g/m<sup>2</sup> Gelatin  
Coating Aid: 7 mg/m<sup>2</sup> N-Oleoyl-N-methyltaurine sodium salt

Matting Agent: 25 mg/m<sup>2</sup> Polymethyl methacrylate  
(mean grain size: 5μ)

TABLE 1

| Sample No.                | Type and Amount of Gelatin Hardener Added to Protective Layer |                                                  |
|---------------------------|---------------------------------------------------------------|--------------------------------------------------|
| 1 (Comparison)            | H-1 (0.5 mmol/gelatin* 100 g)                                 | —                                                |
| 2 (Comparison)            | H-1 (0.75 mmol/gelatin* 100 g)                                | —                                                |
| 3 (Comparison)            | H-1 (1.50 mmol/gelatin* 100 g)                                | —                                                |
| 4 (The present invention) | H-1 (0.5 mmol/gelatin* 100 g)                                 | P-1 (1.2 × 10 <sup>-3</sup> eq./gelatin** 100 g) |
| 5 (The present invention) | H-1 (0.5 mmol/gelatin* 100 g)                                 | P-1 (2.0 × 10 <sup>-3</sup> eq./gelatin** 100 g) |
| 6 (The present invention) | H-1 (0.5 mmol/gelatin* 100 g)                                 | P-1 (2.4 × 10 <sup>-3</sup> eq./gelatin** 100 g) |
| 7 (The present invention) | H-1 (0.75 mmol/gelatin* 100 g)                                | P-1 (0.7 × 10 <sup>-3</sup> eq./gelatin** 100 g) |
| 8 (The present invention) | H-1 (0.75 mmol/gelatin* 100 g)                                | P-1 (1.5 × 10 <sup>-3</sup> eq./gelatin** 100 g) |

H-1 2-Hydroxy-4,6-dichloro-s-triazine sodium salt

\*Amount of gelatin in all layers

\*\*Amount of gelatin in the protective layer

The degree of hardening of each layer was measured as follows:

Each sample was cut into a piece having a width of 0.5 cm and a length of 4 cm. This piece was soaked in an alkali solution (a 0.2N aqueous solution of sodium hydroxide) maintained at 60° C., and the melting time (MT) of each layer was measured.

The film strength was measured as follows:

Each sample was soaked in RD-III Developer as described hereinafter maintained at 35° C. for 25 seconds and, thereafter, a sapphire needle having a diameter of 0.8 mm was pressed to the film surface and moved at a rate of 5 mm/sec. By changing continuously the load on the sapphire needle, the load was determined at which the film was broken or scratches were formed. This load (grams) was used to indicate the film strength.

Samples 1 to 8 as prepared hereinbefore were exposed to light for 1/20 second by the use of the usual tungsten sensitometer and, thereafter, were developed with a developer at 32° C. for 40 seconds, fixed, and washed with water. With the thus-processed samples, the maximum density was measured.

The development processing liquid as used in the above development was a developer RD-III for a super-rapid processing Fuji X-ray automatic developing machine (produced by Fuji Photo Film Co., Ltd.). As a fixing liquid, a fixing solution Fuji F for an X-ray automatic developing machine (produced by Fuji Photo Film Co.) was used.

The results are shown in Table 2 below.

TABLE 2

| Sample No.                | Melting Time (sec)* |                | Film         |                 |
|---------------------------|---------------------|----------------|--------------|-----------------|
|                           | Protective Layer    | Emulsion Layer | Strength (g) | Maximum Density |
| 1 (Comparison)            | 8                   | 8              | 35           | 3.18            |
| 2 (Comparison)            | 43                  | 43             | 45           | 2.78            |
| 3 (Comparison)            | 278                 | 278            | 87           | 2.06            |
| 4 (The present invention) | 280                 | 10             | 35           | 3.18            |
| 5 (The present invention) | 351                 | 9              | 36           | 3.10            |
| 6 (The present invention) | 393                 | 13             | 37           | 3.02            |
| 7 (The present invention) | 257                 | 39             | 47           | 2.82            |
| 8 (The present invention) | 364                 | 47             | 48           | 2.78            |

\*0.2 N NaOH, 60° C.

As can be seen from Table 2, in Samples 1 to 3, the melting time of the protective layer is equal to that of

25 the emulsion layer, whereas, in Samples 4 to 8, the melting time of the protective layer is greater than that of the emulsion layer. The film strength corresponds to the melting time of the emulsion layer, and even if the melting time of the protective layer is increased, no great change in the film strength is observed. Within the film strength range of the samples, no practical problem arises. Furthermore, it can be seen that the maximum density is correlated with the melting time of the emulsion layer and can be controlled independently from the melting time of the protective layer.

30 In order to examine the formation of scum in a fixing solution, a small automatic developing machine produced by Fuji Photo Film Co., Ltd. (sold under the trade name of Fuji X-Ray Processor RE-3; capacity of developer: 2,000 ml; capacity of fixer: 2,000 ml) was used. After passage of 200 sheets having a width of 8.5 cm and a length of 30 cm, the turbidity in each processing liquid and the degree of contamination of the processed film were observed. The degree of contamination of the processed film (the degree of formation of scum) was indicated in the following four grades:

- 35 A: Until 200 sheets were all processed, no contamination was observed.  
 B: When 150 or more sheets were processed, slight contamination was observed.  
 C: When 100 or more sheets were processed, the formation of scum was somewhat observed.  
 D: When 25 or more sheets were processed, the considerable formation of scum was observed.

40 The degree of the turbidity in the processing liquid after processing 200 sheets was indicated in the following three grades:

- xx: Considerable turbidity was observed.  
 x: Slight turbidity was observed.

45 o: No turbidity was observed.

In addition, the amount of gelatin eluted into the development processing liquid was measured by subjecting the liquid to molecular weight fractionation by means of gel chromatography (filler, CephaG-50).

50 The amount of gelatin contained in 100 ml of the development processing liquid was indicated in terms of milligram.

The results are shown in Table 3.

TABLE 3

| Sample No.                | Scum               |                                                               | Amount of Eluted Gelatin (mg, in 100 ml of developer) | Melting Time (0.2 N, NaOH, 60° C.) (sec) |                |
|---------------------------|--------------------|---------------------------------------------------------------|-------------------------------------------------------|------------------------------------------|----------------|
|                           | Turbidity of Fixer | Contamination of Processed Film (degree of formation of scum) |                                                       | Protective Layer                         | Emulsion Layer |
| 1 (Comparison)            | xx                 | D                                                             | 290                                                   | 8                                        | 8              |
| 2 (Comparison)            | x                  | C-D                                                           | 185                                                   | 43                                       | 43             |
| 3 (Comparison)            | o                  | A-B                                                           | 110                                                   | 278                                      | 278            |
| 4 (The present invention) | o                  | A-B                                                           | 112                                                   | 280                                      | 10             |
| 5 (The present invention) | o                  | A                                                             | 90                                                    | 351                                      | 9              |
| 6 (The present invention) | o                  | A                                                             | 85                                                    | 393                                      | 13             |
| 7 (The present invention) | o                  | A-B                                                           | 115                                                   | 257                                      | 39             |
| 8 (The present invention) | o                  | A                                                             | 91                                                    | 364                                      | 47             |

It can be seen from Table 3 that even though the melting time of the emulsion layer is almost the same, as the melting time of the protective layer is increased, the amount of gelatin eluted is decreased and the formation of scum is greatly reduced and, thus, that the scum properties are greatly improved.

#### EXAMPLE 2

Samples 9 to 16 having the same construction as in Example 1 were prepared in which the type of hardener was changed and the hardener was added in the amount shown in Table 4. They were processed in the same manner as in Example 1, and the results are shown in Tables 5 and 6.

TABLE 4

| Sample No.                 | Type and Amount of Gelatin Hardener Added        |                                 |
|----------------------------|--------------------------------------------------|---------------------------------|
|                            | Protective Layer                                 | Emulsion Layer                  |
| 9                          | —                                                | H-2* (0.5 mmol/gelatin** 100 g) |
| 10                         | —                                                | H-2 (0.75 mmol/gelatin** 100 g) |
| 11                         | —                                                | H-2 (1.50 mmol/gelatin** 100 g) |
| 12 (The present invention) | P-1 ( $1.2 \times 10^{-3}$ eq./gelatin*** 100 g) | H-2 (0.5 mmol/gelatin** 100 g)  |
| 13 (The present invention) | P-1 ( $2.0 \times 10^{-3}$ eq./gelatin*** 100 g) | H-2 (0.5 mmol/gelatin** 100 g)  |
| 14 (The present invention) | P-1 ( $2.4 \times 10^{-3}$ eq./gelatin*** 100 g) | H-2 (0.5 mmol/gelatin** 100 g)  |
| 15 (The present invention) | P-1 ( $0.7 \times 10^{-3}$ eq./gelatin*** 100 g) | H-2 (0.75 mmol/gelatin** 100 g) |
| 16 (The present invention) | P-1 ( $1.5 \times 10^{-3}$ eq./gelatin*** 100 g) | H-2 (0.75 mmol/gelatin** 100 g) |

\*H-2: Bis( $\alpha$ -vinylsulfonylacetamido)ethane

\*\*Amount of gelatin in all layers

\*\*\*Amount of gelatin in the protective layer

TABLE 5

| Sample No. | Melting Time (0.2 N NaOH, 60° C.) (sec) |                | Film Strength (g) | Maximum Density |
|------------|-----------------------------------------|----------------|-------------------|-----------------|
|            | Protective Layer                        | Emulsion Layer |                   |                 |
| 25         | 9                                       | 48             | 45                | 3.72            |
|            | 10                                      | 135            | 63                | 3.27            |
|            | 11                                      | 480            | 108               | 2.41            |
| 30         | 12 (The present invention)              | 331            | 47                | 3.68            |
|            | 13 (The present invention)              | 462            | 50                | 3.66            |
|            | 14 (The present invention)              | 530            | 46                | 3.67            |
|            | 15 (The present invention)              | 437            | 67                | 3.25            |

16 (The present invention) 523 139 65 3.20

TABLE 6

| Sample No.                 | Scum               |                                 | Amount of Eluted Gelatin (mg, in 100 ml of developer) | Melting Time (0.2 N NaOH, 60° C.) (sec) |                      |
|----------------------------|--------------------|---------------------------------|-------------------------------------------------------|-----------------------------------------|----------------------|
|                            | Turbidity of Fixer | Contamination of Processed Film |                                                       | Protective Layer (sec)                  | Emulsion Layer (sec) |
| 9                          | x                  | C-D                             | 193                                                   | 48                                      | 48                   |
| 10                         | x                  | C                               | 133                                                   | 135                                     | 135                  |
| 11                         | o                  | A                               | 82                                                    | 480                                     | 480                  |
| 12 (The present invention) | o                  | A-B                             | 96                                                    | 331                                     | 45                   |
| 13 (The present invention) | o                  | A                               | 82                                                    | 462                                     | 47                   |
| 14 (The present invention) | o                  | A                               | 78                                                    | 530                                     | 51                   |

TABLE 6-continued

| Sample No.<br>9               | Scum                       |                                           | Amount of<br>Eluted Gelatin<br>(mg, in 100 ml<br>of developer)<br>193 | Melting Time (0.2 N<br>NaOH, 60° C.) (sec) |                                  |
|-------------------------------|----------------------------|-------------------------------------------|-----------------------------------------------------------------------|--------------------------------------------|----------------------------------|
|                               | Turbidity<br>of Fixer<br>x | Contamination of<br>Processed Film<br>C-D |                                                                       | Protective<br>Layer<br>(sec)<br>48         | Emulsion<br>Layer<br>(sec)<br>48 |
| 15 (The present<br>invention) | o                          | A                                         | 84                                                                    | 437                                        | 130                              |
| 16 (The present<br>invention) | o                          | A                                         | 77                                                                    | 523                                        | 139                              |

As apparent from the above results, in the present invention, the film strength and the maximum density are correlated not with the melting time of the protective layer, but with the melting time of the emulsion layer. Furthermore, it can be seen from Table 6 that as the melting time of the protective layer is increased, the amount of gelatin eluted into the development processing liquid is reduced, which leads to a great improvement in scum properties.

While the invention has been described in detail and with reference to specific embodiments thereof, it will be apparent to one skilled in the art that various changes and modifications can be made therein without departing from the spirit and scope thereof.

What is claimed is:

1. A silver halide light-sensitive photographic material, comprising:

a support; and

a plurality of layers on at least one side of the support wherein at least one of the layers is a light-sensitive silver halide emulsion layer, and further wherein a light-insensitive uppermost layer of the layers has a melting time greater than that of the light-sensitive silver halide emulsion layer, wherein the light-insensitive uppermost layer comprises gelatin hardened by a non-diffusible polymeric hardener.

2. The silver halide light-sensitive photographic material as claimed in claim 1, wherein the relation between the melting time of the uppermost layer (MTu) and that of the light-sensitive silver halide emulsion layer (MTs) represented by MTu/MTs ratio is in a range of more than 1 and less than 20.

3. The silver halide light-sensitive photographic material as claimed in claim 1, wherein the relation between the melting time of the uppermost layer (MTu) and that of the light-sensitive silver halide emulsion layer (MTs) represented by MTu/MTs ratio is in a range of more than 1 and less than 10.

4. The silver halide light-sensitive photographic material as claimed in claim 1, wherein the uppermost layer has a thickness of from about 0.5 to about 2.0 microns.

5. The silver halide light-sensitive photographic material as claimed in claim 1, wherein at least one of the light-sensitive silver halide emulsion layer is provided on both sides of the support and the uppermost layer is provided on the outside of the outermost silver halide emulsion layer existed on both sides of the support.

6. The silver halide light-sensitive photographic material as claimed in claim 1, wherein the plurality of layers contain non-diffusible polymeric hardeners.

7. The silver halide light-sensitive photographic material as claimed in claim 6, wherein the non-diffusible polymeric hardener has molecular weight of more than about 10,000 and at least one functional group reactive to gelatin to form cross-linking.

15 8. The silver halide light-sensitive photographic material as claimed in claim 6, wherein the non-diffusible polymeric hardener has a repeating unit of the formula (I):



20 wherein A is a monomer unit prepared by copolymerizing copolymerizable ethylenically unsaturated monomers; R<sub>1</sub> is hydrogen or a lower alkyl group having 1 to 6 carbon atoms; Q is  $-\text{CO}_2-$ ,



25 30 wherein R<sub>1</sub> is the same as defined above, or an arylene group having 6 to 10 carbon atoms; L is a divalent group having 3 to 15 carbon atoms and containing at least one linking group selected from the members consisting of  $-\text{CO}_2-$  and



35 40 wherein R<sub>1</sub> is the same as defined above, or a divalent group having 1 to 12 carbon atoms and containing at least one linking group selected from the members consisting of  $-\text{O}-$ ,



45 50 55 60 wherein R<sub>1</sub> is the same as defined above; R<sub>2</sub> is  $-\text{CH}=\text{CH}_2$  or  $-\text{CH}_2\text{CH}_2\text{X}$  wherein X is a group capable of being substituted with a nucleophilic group or a group capable of being released in the form of HX upon a base; and x and y each represents molar percent, x being between 0 and 99 and y being between 1 and 100.

65 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 87

polymeric hardener has a repeating unit of the formula (II):



(II)

5

10

wherein A is a polymerized  $\alpha,\beta$ -ethylenically unsaturated addition polymerizable monomer or a mixture of such polymerizable monomers, x is a molar unit of from 10 to 95, and y is a molar unit of from 5 to 90, L is a linking group selected from the group consisting of alkylene, arylene, COZ and COZR<sub>3</sub>, R<sub>3</sub> is selected from the group consisting of alkylene and arylene, Z is O or NH, R is hydrogen or alkyl having 1 to 6 carbon atoms, and R' is  $-\text{CH}=\text{CHR}_2$  or  $-\text{CH}_2\text{CH}_2\text{X}$  where X is a leaving group which can be displaced by a nucleophile or can be eliminated in the form of HX upon treatment with base and R<sub>2</sub> is hydrogen, alkyl or aryl.

15

20

10. The silver halide light-sensitive photographic material as claimed in claim 6, wherein the non-diffusible polymeric hardener contains (i) 5 to 100 molar percent of a repeating unit of the general formula (III):



(III)

wherein R is a hydrogen atom or an alkyl group having 1 to 6 carbon atoms; L, if present, is a divalent linking group having 1 to 20 carbon atoms; X is an active carboxylic ester group; and m is 0 or 1; and optionally contains (ii) 0 to 95 molar percent of one or more other monomer unit "A".

11. The silver halide light-sensitive photographic material as claimed in claim 6, wherein the non-diffusible polymeric hardener has a repeating unit selected from the group consisting of:



-continued



-continued



and



wherein M is a hydrogen atom, a sodium atom or a potassium atom, and x and y represent molar percent x being from 0 to 99, and y being from 1 to 100.

12. The silver halide light-sensitive photographic material as claimed in claim 6, wherein the non-diffusible polymeric hardener is a member selected from the group consisting of [2-(3-vinylsulfonyl)propionyloxy]ethyl ethyl acrylate/sodium acrylamido-2-methylpro-

panesulfonate copolymer, 2-[3-(chloroethylsulfonyl)propionyloxy]ethyl acrylate/sodium acrylamido-2-methylpropanesulfonate copolymer, [3-(chloroethylsulfonyl)propionyloxy]aminomethylstyrene/sodium acrylamido-2-methylpropanesulfonate copolymer and 1-{[2-(4-vinylbenzenesulfonyl)ethyl]sulfonyl}-3-chloroethylsulfonyl-2-propanol/sodium acrylate copolymer.

\* \* \* \* \*

30

35

40

45

50

55

60

65